

# UNITED STATES PATENT OFFICE.

MAXIME J. MARCOTTE, OF ST. LOUIS, MISSOURI.

## IMPROVEMENT IN COMPOSITIONS FOR JOURNALS AND BEARINGS.

Specification forming part of Letters Patent No. 117,652, dated August 1, 1871.

*To all whom it may concern:*

Be it known that I, MAXIME J. MARCOTTE, of the city and county of St. Louis and State of Missouri, have invented a certain new and useful Compound Metal for Journal-Boxes, of which the following is a specification:

My composition consists of certain metals in about the proportions hereinafter named for the formation of the bearing-surface in journal-boxes, and it is intended to diminish the friction between the shaft and the box to such an extent as to render the application of a liquid lubricant, such as oil, almost or entirely unnecessary.

My composition consists of the following metals mixed in about the proportions named, viz: Tin, sixteen pounds; lead, twelve pounds; copper, eight pounds; zinc, eight pounds; antimony, four pounds; finely-pulverized plumbago, one pound.

The tin, copper, zinc, and antimony are first melted together, and, when they are thoroughly mixed, are run into a mold.

When it is desired to fill the journal-boxes, the

ingot taken from the mold is remelted in an iron pot over a slow fire of charcoal or gas-coke. When the ingot is melted the lead and plumbago are thoroughly stirred in, the lead becoming melted and the plumbago thoroughly mixed, resulting in a pasty mass. The journal-box castings are, before filling, heated to the same temperature as the semi-fluid alloy, with which the chambers in the castings are then filled by means of a trowel or other suitable tool, and the journal-face is shaped by means of a smooth cylinder of hard wood of the same diameter as the journal.

I claim as my invention—

The metallic composition, substantially as described.

In testimony of which invention I have hereunto set my hand.

MAXIME J. MARCOTTE.

Witnesses:

SAML. KNIGHT,  
HENRY G. ISAACS.